

## UNITED STATES PATENT OFFICE

1,947,530

## NITRATED SUGAR EXPLOSIVE

Harold A. Lewis, Woodbury, N. J., assignor to  
E. I. du Pont de Nemours & Company, Wil-  
mington, Del., a corporation of Delaware

No Drawing. Application December 22, 1931  
Serial No. 582,649

14 Claims. (Cl. 52—13)

My invention relates to new explosive compositions and more particularly to those comprising nitrated ketoses in solutions of nitric esters.

Most of the commercial explosives in use at the present time contain nitroglycerin as the main explosive ingredient, or, in the case of ammonium nitrate explosives, as the sensitizer of the explosive.

It has frequently been the practice in recent 10 years in the manufacture of dynamites to add various organic materials to the nitroglycerin, or to dissolve them in it for the purpose of controlling the properties of the explosive. Materials dissolved in nitroglycerin have served as 15 freezing point depressants, and the like. Among the compounds added to nitroglycerin for this purpose have been nitrocompounds such as trimitrotoluene, also tetranitroglycerin, ethylene glycol dinitrate, nitrated sugars, and like compounds. The foregoing compounds, being explosives themselves, have had the desired effect 20 on the properties of the explosives, without detracting from the strength.

The use of nitrated sugars dissolved in nitroglycerin, as the explosive oil, has the additional 25 advantage of lowering the cost of the finished explosive. Nitrated sugars, however, have the disadvantage of a lesser degree of stability in nitroglycerin, so that precautions need to be 30 taken with explosives containing nitrated sugars in solution in nitroglycerin.

The kind of sugar used in nitroglycerin explosives has been, in general, cane sugar or sucrose, because of its availability and low price. Sucrose is a disaccharide having a formula commonly accepted as:



Other sugars, glucose for example, have been used also, the formula generally assigned to this compound being:  $\text{CH}_2\text{OH}-(\text{CHOH})_4-\text{CHO}$ .

The above named sugars may be considered as aldoses, and contain the aldehydic group in their formulas.

The use of nitrated aldose sugars, together with nitroglycerin, has been found to be particularly 50 undesirable in gelatin dynamite compositions, because of the effect of the instability of the nitrated sugar in causing a breaking down of the gel and exudation of the liquid explosive ingredient. Various means have been resorted to in an 55 attempt to remedy this undesirable effect and

make such nitrated sugars satisfactory for use in gelatinized explosives. For example, Moran, in U. S. Patent 1,583,895, discloses an improved explosive by utilizing, in place of sugars, glucosides, which are commonly obtained by reactions of sugars with alcohols.

I have discovered that an improved and more stable explosive oil is obtained, if the sugar used has a ketonic rather than an aldehydic linkage in its formula. As an example of such a ketose, 65 I prefer to use levulose, otherwise known as fructose, having the structural formula usually expressed as follows:



While levulose may be obtained, together with other sugars, by the hydrolysis of cane sugar, a more convenient and satisfactory commercial method of production is by the hydrolysis of inulin, which yields levulose alone. Inulin appears naturally in the tubers of the dahlia, Jerusalem artichoke, and others of the Composite, and is readily available from such sources.

My new explosive composition is obtained by dissolving levulose in glycerin, glycol, glycerin-glycol solutions, or similar solvents, and then nitrating the solution obtained. While the solution of levulose in glycerin alone gives a satisfactory explosive oil after nitration, I prefer to use as a solvent glycerin-glycol mixtures, since 85 the solubility of levulose is greater in such mixtures. In this case also, the increased viscosity due to the dissolving of the sugar is compensated for by the lower viscosity of the original mixture, due to the presence of the ethylene glycol.

As illustrative examples of levulose solutions in glycerin, or in glycerin-glycol mixtures, which

are adapted for satisfactory nitration, and without in any way limiting my invention, the following are given:

|                 | 80% | 50% | 70% |
|-----------------|-----|-----|-----|
| Glycerin        |     |     |     |
| Ethylene glycol | 20  |     |     |
| Diglycerin      |     | 20  |     |
| Levulose        | 20  | 30  | 10  |

While I have indicated that levulose is the only sugar in the foregoing examples, it is to be understood that it may be replaced in part, as desired, by sucrose, or other sugars.

My improved explosive oil is not intended for

use alone as an explosive, but will function in the same manner as does nitroglycerin in the usual dynamite compositions. As examples of such compositions, the following will serve, the term nitroglycerin here being intended to cover solutions of levulose in nitroglycerin, such as have just been described.

|                   |      |      |
|-------------------|------|------|
| Nitroglycerin     | 40.0 | 32.0 |
| Nitrocellulose    | 46.0 | 0.7  |
| Sodium nitrate    | 13.0 | 55.0 |
| Wood pulp         | 1.0  | 11.3 |
| Calcium carbonate |      | 1.0  |

In the above formulæ, it should be understood that ammonium nitrate may be used, if desired, in place of nitroglycerin to furnish a portion of the explosive strength, and that various other changes may be made in the details of the ingredients and their proportions. I intend to be limited in my invention only as indicated in the following patent claims:

I claim:

1. An explosive comprising a nitrated ketose free from nitrated aldoses in solution in a liquid nitric ester.
2. An explosive comprising nitrated levulose free from nitrated aldoses in solution in a liquid nitric ester.
3. An explosive comprising a nitrated ketose free from nitrated aldoses in solution in nitroglycerin.
4. An explosive comprising nitrated levulose free from nitrated aldoses in solution in nitroglycerin.
5. An explosive comprising 5 to 40 parts of nitrated levulose free from nitrated aldoses in 95 to 60 parts of a liquid nitric ester.
6. An explosive comprising 5 to 40 parts of

nitrated levulose free from nitrated aldoses in 95 to 60 parts by weight of nitroglycerin.

7. A dynamite composition comprising a liquid explosive consisting of a nitrated ketose in solution in a nitric ester and an absorbent material. 80

8. A dynamite composition comprising a liquid explosive consisting of nitrated levulose in solution in a nitric ester and an absorbent material.

9. A dynamite composition comprising a liquid explosive consisting of nitrated levulose in solution in nitroglycerin and an absorbent material. 85

10. A dynamite composition comprising a liquid explosive consisting of nitrated levulose in 90 solution in nitroglycerin, an oxygen containing salt, and a carbonaceous combustible absorbent material.

11. A gelatinized explosive composition comprising a liquid explosive consisting of a nitrated 95 ketose in solution in a nitric ester, nitrocellulose, an oxygen containing salt, and a carbonaceous combustible absorbent material.

12. A gelatinized explosive composition comprising a liquid explosive consisting of a nitrated 100 levulose in solution in a nitric ester, nitrocellulose, an oxygen containing salt, and a carbonaceous combustible absorbent material.

13. A gelatinized explosive composition comprising a liquid explosive consisting of a nitrated 105 levulose in solution in nitroglycerin, nitrocellulose, an oxygen containing salt, and a carbonaceous combustible absorbent material.

14. A dynamite composition comprising a liquid explosive containing 5 to 40 parts of a nitrated 110 ketose, 95 to 60 parts of a liquid nitric ester, and an absorbent material.

HAROLD A. LEWIS.

40

115

45

120

50

125

55

130

60

135

65

140

70

145

75

150